

Patented Nov. 17, 1925.

1,562,145

# UNITED STATES PATENT OFFICE.

CLARENCE P. BYRNES, OF SEWICKLEY, PENNSYLVANIA.

## COMPOUND METAL AND METHOD OF MAKING THE SAME.

No Drawing.

Application filed March 1, 1921. Serial No. 448,897.

To all whom it may concern:

Be it known that I, CLARENCE P. BYRNES, a citizen of the United States, residing at Sewickley, in the county of Allegheny and State of Pennsylvania, have invented a new and useful Compound Metal and Method of Making the Same, of which the following is a full, clear, and exact description.

My invention relates to the compounding 10 of metals or alloys and is designed to provide a new metal article or product of this nature and also an improved method of making the same.

In wrought iron products the metal is 15 admixed with slag, the metal granules being drawn out in rolling and interlaced with slag filaments having a substantially even distribution among the metal layers.

My invention is aimed to produce a compound metal product in which granules of one metal or alloy are surrounded by another metal or alloy, the granules being preferably welded together so that when worked by compressing or squeezing, forging, rolling, 25 etc., the compound article would have the physical character of wrought iron in that the drawn out granules of one metal will be interspersed with drawn out filaments or portions of another metal or alloy.

In carrying out the method I preferably take a metal or alloy of relatively high melting point such as the product of a steel-making operation, and pour it into a molten bath of another metal or alloy having a 30 lower melting point and a sufficiently low

temperature to granulate the entering stream of the higher melting point metal or alloy. The bath of lower melting point metal or alloy is preferably of sufficiently larger 35 volume and of such a temperature that when equilibrium of temperature is established, the granules of higher melting point metal or alloy are at a welding temperature. If desirable, during the granulating operation 40 the temperature of the bath may be kept from rising too high by feeding in cold or partly heated portions of the bath metal or alloy.

In this operation the granules of the metal 50 poured in collect in a mass in the lower part of the bath if the bath is of less specific gravity than the metal poured in and a mass or ball somewhat similar to a puddle ball will be formed in the lower portion of the bath, this taking the shape of the receptacle.

The excess metal or alloy of the bath be-

neath the surface of which the ball is formed, may be then tapped off or poured off and the mixed mass of metal granules and bath metal may be compressed or squeezed either 60 in the receptacle or mold in which the granulating-mixing operation is carried out, or by discharging the mass and taking it to a squeezer or press.

If, on reaching equilibrium of temperature, 65 the granulated metal is not up to the welding temperature, the temperature of the bath may be raised for bringing the granules to such temperature.

After the squeezing or pressing operation, 70 the metal may be rolled out in the ordinary manner to produce a wrought, compound metal product.

Instead of granulating the one metal or alloy by pouring it in the bath of the other 75 metal or alloy, it may be granulated prior to mixing the two in any desired way, such as by centrifugal force, jet action, etc. The granules, while still hot, are then preferably fed into the bath of the other metal or alloy 80 with or without being preheated.

As an example of the metal, steel may thus be poured into a molten bath of aluminum, copper or aluminum-bronze. Lead or zinc may also be used for the molten bath. 85

If desired, the bath may be provided with a protective layer of slag or glass-like composition to protect the molten bath from oxidation. The operation may also be carried out in a non-oxidizing atmosphere if 90 desired.

If the metals or alloys to be mixed are not of sufficiently different melting point to granulate the one by pouring in a bath of the other, one of them may be granulated 95 separately and the granules fed into the bath of the other.

While I prefer to weld the granules of the one metal together, particularly in the case of iron or steel granules, with some metals 100 or in some cases this may not be necessary as the granules may be cemented or held together by the other metal or alloy forming the bath when the latter is cooled.

In some cases I may use a colder layer of 105 slag or glass-like composition above the molten bath and granulate the other metal by pouring into this cooler slag layer, the granules then descending into the molten metal bath beneath.

The advantages of my invention will be apparent to those skilled in the art since 110

compound metal articles may thus be easily and cheaply formed in which the granules or worked or drawn out granules of one metal are mixed with another metal which 5 may be of an anti-corrosive or protective nature. This method may also be used for making compound metals for non-slip stair-tread, and for other purposes either ornamental or useful.

10 More than two metals or alloys may be thus combined. Any metal or alloy may be used for either or all of the constituents, the method of granulating and mixing may be varied, and other changes may be made without departing from my invention.

By the word "metal" in the claims I intend to cover either a substantially pure metal or an alloy, or a metalloid or semi-metal or alloy thereof. Thus a metal such 20 as steel may be poured into an alloy of iron or steel with another metal or metalloid, such alloy having a lower melting point than the steel to give the granulating and mixing.

I claim:

25 1. A metal product, comprising metal of a relatively high melting point cooled from a molten condition and containing granules of a higher melting point metal arranged in the relation to each other and to the lower 30 melting point metal which results from natural gravity settling of the said granules through the lower melting point metal while it is in molten condition.

2. A metal product, comprising metal of 35 a relatively high melting point cooled from a molten condition and containing granules of a higher melting point metal arranged in the relation to each other and to the lower melting point metal which results from natural gravity settling of the said granules 40 through the lower melting point metal while it is in molten condition, said granules being welded directly to each other.

3. A metal product, comprising a metal 45 of lower melting point and less specific gravity cooled from a molten condition and containing granules of a higher melting point, higher specific gravity metal arranged in the relation to each other and to the lower 50 melting point metal resulting from the natural settling of the granules through the lower melting point metal while the same is in molten condition.

4. A metal product, comprising a metal 55 of lower melting point and less specific gravity cooled from a molten condition and containing granules of a higher melting point, higher specific gravity metal arranged in the relation to each other and to the lower 60 melting point metal resulting from the natural settling of the granules through the lower melting point metal while the same is in molten condition, said granules being welded directly to each other.

65 5. The method of making a compound

metal product, consisting of mixing loose granules of one metal with another metal while the latter is in molten condition and causing the latter metal to encase said loose granules while they remain in granular 70 form.

6. The method of making a compound metal product, consisting in feeding granules of a metal of higher melting point through molten metal of a lower melting 75 point and allowing the compound metal mass to set and cool.

7. The method of making a compound metal product, consisting of feeding metal of a high melting point into a bath of another metal having a low melting point at a sufficient low temperature to granulate the first metal, forming a mixed mass therein and compressing the mass.

8. The method of making a compound 85 metal product, consisting of feeding molten iron or steel into a bath of lower melting point and of sufficient volume and sufficient low temperature to granulate the same, forming a mixed mass of metal in the bath 90 and compressing the mass.

9. The method of making a compound metal product, consisting of feeding molten iron or steel into a bath of lower melting point and of sufficient volume and sufficient 95 low temperature to granulate the same, forming a mixed mass of metal in the bath, removing the surplus molten metal and compressing the mass.

10. The method of making a compound 100 metal product, consisting in feeding granules of a metal of higher melting point through a metal of lower melting point while the latter is in molten condition, allowing the compound metal mass to set and 105 cool, and compressing the same.

11. The method of making a compound metal product, consisting in feeding granulated metal of higher specific gravity 110 through molten metal of lower specific gravity while the latter is in molten condition, removing surplus molten metal, and allowing the remaining compound metal to chill and set.

12. The method of making a compound metal product, consisting in mixing loose granules of metal of higher melting point with a metal of lower melting point while the latter is in molten condition and causing the latter metal to encase the said loose 120 granules while they remain in granular form.

13. The method of making a compound metal product, consisting in mixing loose 125 granules of metal of higher melting point with a metal of lower melting point while the latter is in molten condition and causing the latter metal to encase the said loose granules at the welding temperature of the granules of the higher melting point metal. 130

14. The method of making a compound metal product, consisting in mixing loose granules of metal of higher melting point with a metal of lower melting point while

5 the latter is in molten condition and causing the latter metal to encase the said loose granules while they remain in granular form, and then compressing the same.

15. The method of making a compound metal product, consisting in feeding granules of higher melting point metal into a bath of lower melting point metal, causing said granules to weld directly to each other, and allowing the bath metal to cool and set.

15 16. The method of making a compound metal product, consisting in feeding gran-

ules of higher melting point metal into a bath of lower melting point metal under non-oxidizing conditions, and allowing the latter metal to cool and set while enveloping 20 the granules.

17. The method of making a compound metal product, consisting in feeding granules of higher melting point metal into a bath of lower melting point metal, causing said granules to weld directly to each other, allowing the bath metal to cool and set, and then compressing.

In testimony whereof, I have hereunto set my hand.

CLARENCE P. BYRNES.